

# United States Patent [19]

Iwama et al.

[11] 3,784,383  
[45] Jan. 8, 1974

- [54] **LIGHT SENSITIVE SILVER HALIDE COLOR PHOTOGRAPHIC MATERIAL**
- [75] Inventors: **Masakuni Iwama; Mitsuto Fujiwara; Tamotsu Kojima; Toshihiko Yamamoto**, all of Tokyo, Japan
- [73] Assignee: **Konishiroku Photo Industry Co., Ltd.**, Tokyo, Japan
- [22] Filed: **May 23, 1972**
- [21] Appl. No.: **256,010**
- Related U.S. Application Data**
- [63] Continuation-in-part of Ser. No. 28,083, April 13, 1970, abandoned.
- [30] **Foreign Application Priority Data**
- Apr. 14, 1969 Japan ..... 44-28287
- [52] U.S. Cl. ..... 96/100, 96/9
- [51] Int. Cl. ..... G03c 1/40
- [58] Field of Search ..... 96/100, 9

[56] **References Cited**

- UNITED STATES PATENTS
- |           |         |                      |        |
|-----------|---------|----------------------|--------|
| 3,034,892 | 5/1962  | Gledhill et al. .... | 96/100 |
| 3,459,552 | 8/1969  | Yoshida et al. ....  | 96/100 |
| 3,481,741 | 12/1969 | Yoshida et al. ....  | 96/100 |
| 3,583,971 | 6/1971  | Yoshida et al. ....  | 96/100 |
| 3,642,485 | 2/1972  | Oishi et al. ....    | 96/9   |

3,667,956 6/1972 Iwama et al. .... 96/100

Primary Examiner—J. Travis Brown  
Attorney—Eric H. Waters et al.

[57] **ABSTRACT**

A compound of the formula:



wherein  $n$  is an integer of 1 to 4 and R is a lower alkyl group is found to be useful as a cyan coupler providing auto-masking mechanism for light-sensitive color photographic materials so as to compensate for the deficient color reproductivity of said materials.

**8 Claims, No Drawings**

# LIGHT SENSITIVE SILVER HALIDE COLOR PHOTOGRAPHIC MATERIAL

## CROSS REFERENCE TO RELATED APPLICATIONS

This application is a continuation-in-part application of Ser. No. 28,083, filed Apr. 13, 1970 now abandoned.

This invention relates to a light-sensitive silver halide color photographic material containing a cyan coupler usable in the form of a solution in an organic solvent, said cyan coupler providing auto-masking mechanism for the light-sensitive color photographic material so as to compensate for the deficient color reproductivity of said material.

Almost all of the cyan couplers used as color formers in light-sensitive color photographic materials are compounds of the 1-naphthol-2-carboxylic acid or ortho-aminophenol type. Particularly, cyan colored couplers having an arylazo group at their 4-position have been utilized as colored couplers provided with automasking mechanism so as to compensate for deficiencies in color reproductivity of color photographic materials concerned.

For example, U.S. Pat. No. 3,034,892 discloses auto-masking cyan couplers represented by the formula



wherein X is an integer of 0 to 4, Y is 0 to 1, R<sub>2</sub> is one member selected from the group consisting of phenyl groups, alkyl groups having 6 to 15 carbon atoms, alkyl-substituted phenyl groups and alkyl-substituted phenoxyphenyl groups, and R<sub>3</sub> is a straight chain or branched-chain alkyl group having one to four carbon atoms. The said United States patent describes as an example of said couplers a compound of the formula



This coupler when dispersed in an organic solvent displays quite excellent efficiencies as a protected coupler for light-sensitive silver halide color photographic material. However, the arylazo component of said coupler has to be prepared through very complex steps, and therefore the coupler cannot but become relatively expensive.

In addition, Japanese Patent Publication No. 29,413/1968 corresponding to U.S. Pat. No. 3,459,552 discloses couplers of the formula



wherein R is a lower alkyl group, and R' is a monocyclic aryl group having nine or more carbon atoms and containing at least one alkoxy carbonyl group; Japanese Patent Publication No. 11,304/1967 corresponding to U.S. Pat. No. 3,481,741 discloses couplers of the formula



wherein R' is a branched alkyl group having six or more carbon atoms, and R is a lower alkyl group; U.S. Pat. No. 2,521,908 discloses couplers of the formula



wherein X is a hydrogen atom or an alkyl group, Y is a monocyclic aryl group or an aralkyl group, and R<sub>1</sub> is a monocyclic aryl group, e.g.,



U.S. Pat. No. 2,706,684 discloses couplers of the formula



wherein X is a hydrogen atom or an alkyl group, Y is a monocyclic aryl group in which the ortho-position with respect to the amide group has been substituted by a halogen atom, an alkoxy group or a monocyclic aryl oxy group, and R<sub>1</sub> is a monocyclic aryl group; and Belgian Pat. No. 709,404 discloses couplers of the formula



wherein R<sub>1</sub> and R<sub>2</sub> are individually a hydrogen atom or an alkyl or aryl group, R<sub>3</sub> is an alkyl, alkylene, aryl, amino, alkoxy or aryloxy group, R<sub>4</sub> is a carboxy, aryl oxy, carbonyl, acyl, sulfo or nitro group, and n is 1 to 6.

These couplers, however, when used in light-sensitive color photographic materials have considerably more drawbacks as compared with the aforesaid coupler (I). For example, these couplers have the absorption maximum at a suitable spectral region but the resulting cyan dye images have no desirable color phase as a negative image. Further, it is difficult to find a color sensitizing dye suitable for positive color sensitive material which is to be adapted to said negative image. Still further, the above-mentioned couplers have less of a disadvantage with respect to spectral absorption but are extremely low (about one-half) in emulsion speed as compared with the coupler (I) and inferior in graininess of the resulting color images. Because of their properties, the protected type colored cyan couplers of Japanese Pat. Publication No. 11,304/1967 are used for negative sensitive materials. It is therefore desirable that couplers have such properties that they are excellent in solubil-

ity in organic solvents, favorable in auto-masking effects (broad in the range of isospecific points of blue and green portions), high in speed and prominent in graininess of the resulting images.

5 Couplers having all such properties have, of course, not been provided hitherto, but the coupler (I) has many desirable properties. However, when the coupler (I) is actually dissolved in an organic solvent such as tricresyl phosphate or the like and is finely dispersed in 10 an aqueous gelatin solution, the resulting dispersion is somewhat low in stability and the dispersed particles frequently unite with each other when the dispersion is allowed to stand for a long time. Further, even if the -COCH<sub>3</sub> of the arylazo group is varied to -COC<sub>2</sub>H<sub>5</sub>, 15 -COC<sub>3</sub>H<sub>7</sub> or the like, no substantial change is seen in solubility. Moreover, there is a new disadvantage that if said -COCH<sub>3</sub> is varied to -COC<sub>4</sub>H<sub>9</sub>, the coupler (I) brings about a marked color variation when subjected to ordinary color development and becomes unusable 20 in practice.

The present invention provides couplers which are free from the above-mentioned disadvantages.

That is, the present invention is concerned with light-sensitive silver halide color photographic materials 25 characterized by containing a coupler having the formula



wherein n is an integer of 1 to 4, and R is a lower alkyl group.

45 Concrete examples of the couplers employed in the present invention are as shown below.

1. 1-Hydroxy-4-(2-carboethoxyphenylazo)-N-[δ-(2,4-di-t-amylphenoxy)-butyl]-2-naphthamide



m.p. 169-170°C.

60 2. 1-Hydroxy-4-(2-carbomethoxyphenylazo)-N-[δ-(2,4-di-t-amylphenoxy)-butyl]-2-naphthamide.



m.p. 175-176°C.

3. 1-Hydroxy-4-(2-carbo-n-propyloxyphenylazo)-N-[δ-(2,4-di-t-amylphenoxy)-butyl]-2-naphthamide.



m.p. 128-129°C.

4. 1-Hydroxy-4-(2-carbomethoxyphenylazo)-N-[δ-(2,4-di-t-amylphenoxy)-propyl]-2-naphthamide.



m.p. 188-189°C.

5. 1-Hydroxy-4-(2-carboethoxyphenylazo)-N-[β-(2,4-di-t-amylphenoxy)-ethyl]-2-naphthamide.



m.p. 187-188°C.

6. 1-Hydroxy-4-(2-carbo-n-butoxyphenylazo)-N-[δ-(2,4-di-t-amylphenoxy)-butyl]-2-naphthamide.



m.p. 129-130°C.

7. 1-Hydroxy-4-(2-carboethoxyphenylazo)-N-(2,4-di-t-amylphenoxy)-methyl-2-naphthamide.



m.p. 195-196°C.

40 Synthesis examples of the couplers used in the present invention are set forth below.

Synthesis Example 1

45 Synthesis of 1-hydroxy-4-(2-carboethoxyphenylazo)-N-[δ-(2,4-di-t-amylphenoxy)-butyl]-2-naphthamide (coupler (1)):

50 Into a mixture comprising 220 g. of ethyl aminobenzoate, 400 cc. of concentrated hydrochloric acid and 800 cc. of water was dropped with stirring at 0° ± 5°C. over a period of about 15 minutes a mixture comprising 92 g. of NaNO<sub>2</sub> and 300 cc. of water, and the resulting mixture was stirred at 0° ± 5°C. for 30 minutes to prepare a diazo solution. The thus prepared diazo solution was dropped with stirring at 5° ± 5°C. over a period of 30 minutes into a solution of 600 g. of 1-hydroxy-N-[δ-(2,4-di-t-amylphenoxy)-butyl]-2-naphthamide in 18 liters of pyridine, and the resulting mixture was stirred at below 10°C. for 1 hour.

55 The reaction mixture was charged into 25 liters of water, and the deposited red crystals were recovered by filtration. After washing with water, the crystals were dried and then recrystallized from 55 liters of n-propanol to form a red powder. This red powder was washed with 300 ml. of methanol and then dried to obtain 750 g. of 1-hydroxy-4-(2-carboethoxyphenylazo)-N-[δ-(2,4-di-t-amylphenoxy)-butyl]-2-naphthamide, coupler (1), as a red powder. m.p. 169° - 170°C., yield 92 percent.

## Elementary analysis:

|            | C (%) | H (%) | N (%) |
|------------|-------|-------|-------|
| Calculated | 73.70 | 7.58  | 6.45  |
| Found      | 73.90 | 7.66  | 6.38  |

## Synthesis Example 2

Synthesis of 1-hydroxy-4-(2-carbo-n-propyloxyphenylazo)-N-[ $\delta$ -(2,4-di-t-amylphenoxy)-butyl]-2-naphthamide (coupler (3)):

The same procedures as in Synthesis Example 1 were effected, except that 239 g. of n-propyl o-aminobenzoate was used in place of the ethyl o-aminobenzoate. The resulting red powder was recrystallized from 75 liters of alcohol to obtain 700 g. of 1-hydroxy-4-(2-carbo-n-propyloxyphenylazo)-N-[ $\delta$ -(2,4-di-t-amylphenoxy)-butyl]-2-naphthamide, coupler (3), as a red powder. m.p. 126° - 128°C., yield 83.3 percent.

## Elementary analysis:

|            | C (%) | H (%) | N (%) |
|------------|-------|-------|-------|
| Calculated | 73.95 | 7.72  | 6.21  |
| Found      | 74.06 | 7.59  | 6.15  |

## Synthesis Example 3

Synthesis of 1-hydroxy-4-(2-carbomethoxyphenylazo)-N-[ $\gamma$ -(2,4-di-t-amylphenoxy)-propyl]-2-naphthamide (coupler (4)):

The same procedures as in Synthesis Example 1 were effected, except that 201 g. of methyl o-aminobenzoate was used in place of the ethyl o-aminobenzoate and 582 g. of 1-hydroxy-N-[ $\gamma$ -(2,4-di-t-amylphenoxy)-propyl]-2-naphthamide was used in place of the 1-hydroxy-N-[ $\delta$ -(2,4-di-t-amylphenoxy)-butyl]-2-naphthamide. The resulting red powder was recrystallized from 170 liters of n-propanol to obtain 740 g. of 1-hydroxy-4-(2-carbomethoxyphenylazo)-N-[ $\gamma$ -(2,4-di-t-amylphenoxy)-propyl]-2-naphthamide, coupler (4), as a red powder. m.p. 188° - 189°C., yield 94.3 percent.

## Elementary analysis:

|            | C (%) | H (%) | N (%) |
|------------|-------|-------|-------|
| Calculated | 73.17 | 7.27  | 6.74  |
| Found      | 73.12 | 7.35  | 6.65  |

## Synthesis Example 4

Synthesis of 1-hydroxy-4-(2-carboethoxyphenylazo)-N-[ $\beta$ -(2,4-di-t-amylphenoxy)-ethyl]-2-naphthamide (coupler (5)):

The same procedures as in Synthesis Example 1 were effected, except that 563 g. of 1-hydroxy-N-[ $\beta$ -(2,4-di-t-amylphenoxy)-ethyl]-2-naphthamide was used in place of the 1-hydroxy-N-[ $\delta$ -(2,4-di-t-amylphenoxy)-butyl]-2-naphthamide. The resulting red powder was recrystallized from 75 liters of n-propanol to obtain 750 g. of 1-hydroxy-4-(2-carboethoxyphenylazo)-N-

[ $\beta$ -(2,4-di-t-amylphenoxy)-ethyl]-2-naphthamide as a red powder. m.p. 187° - 188°C., yield 95.5 percent.

## Elementary analysis:

|            | C (%) | H (%) | N (%) |
|------------|-------|-------|-------|
| Calculated | 73.17 | 7.27  | 6.74  |
| Found      | 73.05 | 7.30  | 6.70  |

Excellent properties of the couplers used in the present invention are shown below with reference to test examples.

## Test Example 1

The couplers used in the present invention and other couplers were compared to each other in solubility for tricresyl phosphate in such a manner that 1 g. of each coupler was dissolved at 80°C. in tricresyl phosphate and then allowed to stand at 20°C., and the time required for initiation of the crystallization of said coupler was measured to obtain the results as shown below.

|                     | Amount of tricresyl phosphate used, ml. | Crystallization initiation time, min. |
|---------------------|-----------------------------------------|---------------------------------------|
| Control coupler A   | 25                                      | 2                                     |
|                     |                                         |                                       |
| Control coupler B   | 10                                      | 10                                    |
|                     |                                         |                                       |
| Present coupler (3) | 10                                      | 90                                    |
| Present coupler (6) | 10                                      | 30                                    |

## Test Example 2

Couplers of the present invention which were of the formula shown below and the known coupler of the same formula, except that R' was different, were tested for solubility in a high boiling solvent to obtain the results set forth in the table below. (One gram of each coupler was thoroughly dissolved in tricresyl phosphate and the solubility thereof was represented by the minimum amount (cc.) of the tricresyl phosphate in which the coupler did not deposit at room temperature for more than 24 hours.)



## Bleaching solution:

Red prussiate — 100 g.  
Potassium bromide — 20 g.  
Water to make — 1,000 ml.

5 (pH 6.9 ± 0.3)

## Fixing solution:

Hypo — 200 g.  
Sodium sulfite — 20 g.  
Acetic acid (28 percent) — 45 ml.  
10 Boric acid — 7.5 g.  
Potash alum — 20 g.  
Water to make — 1,000 ml.  
(pH 4.5 ± 0.2)

| R'                            | Known coupler    | Present coupler   |                                 |                                    |                                    |
|-------------------------------|------------------|-------------------|---------------------------------|------------------------------------|------------------------------------|
|                               | -CH <sub>3</sub> | -OCH <sub>3</sub> | -OC <sub>2</sub> H <sub>5</sub> | -O(n)C <sub>3</sub> H <sub>7</sub> | -O(n)C <sub>4</sub> H <sub>9</sub> |
| Amount of tricresyl phosphate | 10               | 15                | 30                              | 10                                 | 12                                 |

The couplers employed in the present invention may be optionally varied in solubility. Moreover, all these couplers are excellent in emulsion property and masking property, and they always give light-sensitive color photographic materials having uniform photographic properties.

The present invention is illustrated in detail below with reference to examples.

## Example 1

1 Part of the coupler (3) was dissolved in 10 parts of 35 tricresyl phosphate (hereinafter abbreviated to T.C.P.) with stirring at 80°C. and this solution was added to 100 parts of a 10 percent aqueous gelatin solution kept at 60°C., and the mixed solution was charged with 2 parts of a 10 percent aqueous sodium alkylbenzenesulfonate solution. Subsequently, the liquid was stirred at about 65°C. for 5 minutes with a high speed rotary mixer. This operation was repeated 5 times at intervals of 1 minute to prepare a coupler dispersion. 13.5 Parts of this dispersion were added with stirring at 35°C. to 100 parts of a light-sensitive silver iodobromide emulsion containing a red light-sensitive sensitizing dye, and the resulting mixture was coated on a film support and then dried to obtain a red light-sensitive color photographic material.

The thus obtained photographic material was exposed to red light through an optical wedge and was subjected to ordinary color development using a color developer of the following composition:

## Color developer:

N,N-Diethyl-p-aminobenzoate — 2.0 g.  
Sodium sulfite — 2.0 g.  
Sodium carbonate (monohydrate) — 500 g.  
Hydroxylamine hydrochloride — 1.5 g.  
Potassium bromide — 1.0 g.  
Water to make — 1,000 ml.  
(pH 10.8 ± 0.1)

Thereafter, the photographic material was bleached and fixed by use of a bleaching solution and a fixing solution of the compositions shown below to remove undeveloped silver halide and by-produced reduced silver.

In the above manner, a cyan colored negative image and a red positive image comprising unreacted residual coupler were obtained. This red positive image showed a sufficient red color and had isospecific points of 405 m $\mu$  and 540 m $\mu$ .

## Example 2

A mixture comprising 1 part of the coupler (3) and 3 parts of 1-hydroxy-N-[δ-(2,4-di-t-amylphenoxy)-butyl]-2-naphthamide was dissolved with stirring at 80°C. in 10 parts of T.C.P., and was added to 100 parts of a 10 percent aqueous gelatin solution kept at 60°C., and the mixed solution was charged with 2 parts of a 10 percent aqueous sodium alkylbenzenesulfonate solution. Subsequently, the liquid was stirred at about 65°C. for 5 minutes by use of a high speed rotary mixer. This procedure was repeated 5 times at intervals of 1 minute to prepare a coupler dispersion. 10 Parts of this coupler dispersion was added to 100 parts of a high speed light-sensitive silver iodobromide emulsion containing a red light-sensitive sensitizing dye, and the resulting mixture was treated in the same manner as in Example 1 to obtain a red light-sensitive color photographic material.

This photographic material was exposed to red light through an optical wedge and was color-developed, bleached and fixed in the same manner as in Example 1, whereby a cyan colored negative image and an excellent red positive image were obtained simultaneously. Transparency also was quite excellent.

## Example 3

Example 2 was repeated, except that di-n-butyl phthalate was used in place of the T.C.P., to obtain a red light-sensitive color photographic material. This photographic material was exposed to red light and then treated in the same manner as in Example 2, whereby a cyan colored negative image and an excellent red positive image were obtained simultaneously.

## Example 4

A mixture comprising 0.3 part of the coupler (1), 0.7 part of the coupler (6) and 3 parts of 1-hydroxy-N-[δ-(2,4-di-t-amylphenoxy)-butyl]-2-naphthamide was

treated in the same manner as in Example 2 to obtain a red light-sensitive color photographic material. This photographic material was exposed to red light and then treated in the same manner as in Example 2, whereby a cyan colored negative image and an excellent red positive image were obtained simultaneously.

## Example 5

This experiment was conducted to compare the photographic properties of a cyan coupler according to the present invention with three cyan couplers of the prior art having a closely related structure.

The couplers tested were as follows:

Present coupler (1)

Control coupler B (Coupler IV, U.S. Pat. No. 3,481,741)

See Test Example 1

Control coupler C (Compound II, U.S. Pat. No. 3,034,892)



Control coupler D (Coupler III, U.S. Pat. No. 3,459,552)



| Colored cyan coupler | Relative speed | Fog  | Gamma | Light* fastness of masking dye | Maximum absorption of masking dye | Maximum absorption of developed color image |
|----------------------|----------------|------|-------|--------------------------------|-----------------------------------|---------------------------------------------|
| (1)                  | 320            | 0.04 | 0.46  | 83%                            | 500m $\mu$                        | 690m $\mu$                                  |
| B                    | 200            | 0.05 | 0.33  | 72"                            | 440-500"                          | 690"                                        |
| C                    | 100            | 0.04 | 0.23  | 60"                            | 506"                              | 690"                                        |
| D                    | 230            | 0.04 | 0.30  | 78"                            | 518"                              | 720"                                        |

\*This value is a percentage of the residual density of the masking dye as compared with the original density of same when an image was subject to a Fado-O-Meter for 50 hours.

Into 10 parts of tricresyl phosphate was dissolved 1.25 parts of coupler (1) with stirring at 80°C., and the solution was added to 100 parts of an aqueous 10 percent gelatin solution that had been preliminarily heated

to 60°C. Two parts of a 10 percent aqueous solution of sodium alkylbenzene sulfonate were added and dispersed with mixing by means of a high speed mixer for 5 minutes at 65°C. followed by stopping the stirring for 1 minute. This was repeated 5 times to give a dispersion of the coupler.

To 100 parts of a red-sensitive silver iodobromide emulsion were added 13.5 parts of the above dispersion with stirring at 35°C. and coated on a film support and dried to give a red-sensitive color photographic material.

The above procedure was repeated using each of control couplers B, C and D to provide dispersions from which red-sensitive color photographic films were prepared as above.

The thus prepared four color photographic sensitive films were exposed to red light using an optical wedge and then subjected to conventional color development using the following color developer.

Color developer:

G.

- 25 N,N-diethyl-para-aminoaniline sulfate — 2.0  
Sodium sulfite — 2.0  
Sodium carbonate (mono-hydrate) — 50.0  
Hydroxylamine hydrochloride — 1.5  
Potassium bromide — 1.0  
30 Water to make 1,000 ml. (pH 10.80.1).  
Thus developed photographic films were bleached and fixed using the bleaching solution and the fixing solution having the following formulas, respectively, to remove the undeveloped silver halide and thus reduced 35 silver.

Bleaching solution:

G.

- 40 Potassium ferricyanide — 100  
Potassium bromide — 20  
Water to make 1,000 ml (pH 6.9 0.3).

Fixing solution:

- Sodium thiosulfate — g. 200  
Sodium Sulfite — g. 20  
Acetic acid (28%) — ml. 45  
Boric acid — g. 7.5  
Potassium alum — g. 20  
Water to make 1,000 ml. (pH 4.5 0.2).

- 50 The photographic properties were as follows:

As can be seen, coupler (1) and coupler C both are 65 equally excellent in spectral characteristics including spectral and maximum absorptions of masking dye and colored dye images. However, the coupler (1) is much

more excellent in speed and light fastness of masking dye than coupler C. Particularly with respect to the speed, coupler (1) is three times faster than coupler C. This means that the coupler (1) is very preferred for auto-masking mechanism when it is jointly used with a colorless coupler. Such an unexpected technical advantage of coupler (1) over coupler C results from the structural difference between the two, in that the azo portion of coupler (1) is of the ester ( $-\text{COOC}_2\text{H}_5$ ) type whereas that of coupler C is of the ketone ( $-\text{COCH}_3$ ) type.

In both coupler (1) and the coupler B, the azo portions are of the ester ( $-\text{COOR}$ ) type, which show good spectral characteristics. However, coupler B disadvantageously has undesired spectral absorption of masking dye, which is due to the inclusion of a branched alkyl group. The emulsion test indicates that coupler B has a broad absorption comprising two absorption maxima at  $440 \text{ m}\mu$  and  $500 \text{ m}\mu$ , as shown below:



This means that coupler B is not appropriate as colored cyan coupler because its masking action is too excessive in the short wavelength region.

Both coupler (1) and coupler D which have the azo portion of the ester type are equally competent in photographic properties. However, coupler D is detrimentally undesirable because of its having a maximum absorption at a very long wavelength site, i.e.,  $720 \text{ m}\mu$ . This is considered to be due to the existence of an anilide moiety at the 2-position of the naphthol nucleus.

Thus it can be seen that the particular structure of the couplers of the present invention provide an unexpected combination of desirable solubility and photographic properties not exhibited by prior art couplers.

What we claim is:

1. A light-sensitive silver halide color photographic material incorporated with a coupler having the formula



wherein  $n$  is an integer of 1 to 4 and R is a lower alkyl group.

2. A light-sensitive silver halide color photographic material as claimed in claim 1, wherein said coupler is a compound of the following structure



3. A light-sensitive silver halide color photographic material as claimed in claim 1, wherein said coupler is a compound of the following structure



4. A light-sensitive silver halide color photographic material as claimed in claim 1, wherein said coupler is a compound of the following structure



5. A light-sensitive silver halide color photographic material as claimed in claim 1, wherein said coupler is a compound of the following structure



15

6. A light-sensitive silver halide color photographic material as claimed in claim 1, wherein said coupler is a compound of the following structure



5

7. A light-sensitive silver halide color photographic material as claimed in claim 1, wherein said coupler is a compound of the following structure



10

8. A light-sensitive silver halide color photographic material as claimed in claim 1, wherein said coupler is a compound of the following structure



15

20

25

30

\* \* \* \* \*

35

40

45

50

55

60

65